

July 10, 1956

E. M. HOLUB ET AL

2,754,234

THERMOCHEMICAL METAL REMOVAL

Filed March 18, 1953

2 Sheets-Sheet 1

*Fig. 1.*



*Fig. 3.*



*Fig. 4.*



*Fig. 2.*



INVENTORS  
EDWARD M. HOLUB  
CARL E. HARTMANN  
BY *Richard S. Schrenk*  
ATTORNEY

*Fig. 5.*

July 10, 1956

E. M. HOLUB ET AL

2,754,234

THERMOCHEMICAL METAL REMOVAL

Filed March 18, 1953

2 Sheets-Sheet 2



Fig. 6



Fig. 7



Fig. 8.

INVENTORS  
EDWARD M. HOLUB  
CARL E. HARTMANN  
BY *Richard S. Shreve*  
ATTORNEY

2,754,234

## THERMOCHEMICAL METAL REMOVAL

Edward M. Helub, Plainfield, and Carl E. Hartmann, North Florham Park, N. J., assignors to Union Carbide and Carbon Corporation, a corporation of New York

Application March 18, 1953, Serial No. 343,034

7 Claims. (Cl. 148—9.5)

This invention relates to thermochemical metal removal, and more particularly to method and apparatus for machine scarfing of hot stainless steel of approximately rolling temperatures and at approximately rolling speeds.

The conditioning of stainless steels has always been a costly and time-consuming process, and is one of the major bottlenecks in the production of stainless steel today. The use of the powder scarfing process has materially aided the reduction of cost and time in stainless steel conditioning, but such powder scarfing has been done on cold workpieces, and at speeds much too slow to keep pace with rolling speeds.

It is, therefore, the main object of the present invention to provide method and apparatus for machine scarfing of hot stainless steel of approximately rolling temperatures and at approximately rolling speeds.

Prior attempts to hot scarf stainless steel were not successful for a number of reasons, one of which is because the hot slag from the scarfing zone projected ahead onto the hot workpiece would adhere tenaciously and virtually weld itself to the hot workpiece to the extent of rendering the process inoperative. By contrast, with a cold workpiece, the hot slag impinging on the cold surface does not adhere but instead is chilled to a brittle or friable state and is comparatively easily removed.

It is, therefore, another object of the present invention to facilitate the removal of hot slag produced in the hot scarfing of stainless steels.

Another problem in the prior attempts to hot scarf stainless steel was the difficulty of distributing the powder over commercial widths for single pass operation, particularly to distribute the powder over a number of outlets so that individual powder streams might be applied to the multiple nozzles of a standard desurfacing machine. When gas-borne powder is conducted horizontally, the powder tends to separate out by gravity, and when passing around a bend the powder tends to separate out by centrifugal force or inertia.

The importance of powder control is reflected in the expensive metal lost by removing too much metal by too deep a cut. Contrary to the expected result, too little powder below a critical degree at any point across the body removes excessive metal along a groove, and too little powder uniformly distributed across the surface results in too deep a cut for economic operation, and produces an undesirably rough, irregular surface. On the other hand, too much powder takes up the oxygen, leaving too little oxygen to burn the steel.

It is, therefore, another object of the present invention to provide improved powder distribution for the hot scarfing of stainless steels.

According to the present invention a refractory metal body, such as a workpiece of stainless steel, is desurfaced by applying preheat to a local surface portion of such body at substantially rolling temperatures, discharging a relatively flat stream of oxidizing gas at an acute angle against such heated portion, discharging a separate rela-

tively flat stream of gas containing uniformly transversely distributed powdered solid fuel at an acute angle toward such oxidizing gas stream, so that such streams form angles with one another and with such surface portion of the body, and relatively moving the body and such streams at substantially rolling speed so that successive surface portions thereof are progressively removed thermochemically by the combined scarfing action of the powdered solid fuel and the oxidizing gas stream. Preferably the powder is supplied to the process by passing a stream of gas containing powdered solid fuel through a distributor wherein it is divided into a plurality of separate equal paths, and discharging the gas-borne powder from said paths through a row of outlets forming a relatively flat stream of gas-borne powder.

Fig. 1 is a diagrammatic view of the apparatus for hot scarfing stainless steel with the use of ferrous metal powder according to, and for carrying out the method of the present invention;

Fig. 2 is a side elevation of the scarfing head shown in Fig. 1;

Fig. 3 is a detail section of the powder distributor;

Fig. 4 is a cross section taken along the line 4—4 of Fig. 3;

Fig. 5 is a detail section of the air injector;

Fig. 6 is a front elevation of a desurfacing head similar to Fig. 1 but showing a modification;

Fig. 7 similarly shows a further modification; and

Fig. 8 shows the provision for scarfing the under side 30 of a workpiece, and for scarfing four sides simultaneously.

As shown in the drawings, the illustrated scarfing apparatus S is mounted on a suitable support above the path of the work W, such as a hot slab of stainless steel to be scarfed at substantially rolling temperatures and speeds. The apparatus S includes a relatively flat powder nozzle 10 mounted on a modified scarfing head 12 having a plurality of flat slotted nozzles 14 for discharging a relatively flat stream 20 of commercially pure oxygen against the work W, as well as upper and lower rows of ports 16 and 18 for discharging preheating gas flames adjacent such scarfing oxygen stream. The preheating gas flames 22 and 24 extend above and below the oxygen stream 20, forming dihedral angles with the work surface 25.

Oxygen is supplied to the head 12 and slotted nozzles 14 from a suitable source of oxygen under pressure. At the same time, a suitable combustible gas is supplied to the preheating flame ports 16 and 18. The powder nozzle 10 is mounted directly on the blowpipe nozzle head 12, and comprises a metal base 34 and a metal cover 36 suitably bolted together. The base 34 and the cover 36 have convergent inner walls as shown in Fig. 2 and are provided with a channel or mating channels which have divergent sides but parallel axes as shown in Fig. 1, forming closely and uniformly spaced slots 39 for discharging a suitable relatively flat powder-laden carrier gas stream 40, which can be any suitable gas, such as air, nitrogen or oxygen for example. The discharge face of the powder nozzle 10 is positioned on the blowpipe nozzle head 12 so that the slots discharge the separate powder laden carrier gas streams from flat orifices 41 located above the front upper edge of the nozzle 12. These streams combine to form the transversely continuous powder laden gas stream 40 which forms a dihedral angle with the oxygen stream 20, and with the work surface 25.

Each of the slots 39 is in connection with an individual branch tube 42 of a battery of such tubes leading from a distributor 44, which in turn is connected to a powder laden gas supply line 45. The line 45 is provided with a booster 46, another booster 47, an air op-

erated pinch valve 48, and is finally connected to a powder dispenser 50 of standard or conventional construction.

The distributor 44 is shown in detail in Figs. 3 and 4 and comprises a cylindrical shell 52 provided with a hollow insert 43, having in its top a central inlet 53 connected to the supply line 45. The base of the shell 52 has inserted thereon a rubber plug 51, and a group of outlets 54 is annularly uniformly spaced therearound and respectively connected to the branch tubes 42. The insert 43 is locked in position to provide a distributing chamber therebelow, in which the plug 51 forms a cushion for the incoming powder stream being distributed to the branch tubes 42.

The boosters 46 and 48 are shown in detail in Fig. 5, and each comprises an entrance jacket 55 surrounding the powder laden line 45 and having a compressed air inlet 56 connected to a suitable source of air under pressure. Within the jacket 55, the air-powder line 45 is drilled on a long angle in the direction of movement, forming uniformly distributed bores 57 which direct the additional air in the direction to increase the velocity, and in the case of the booster 46, to aid the distribution of the powder.

As shown in Fig. 1, there is provided a water supply nozzle 58 for discharging a flat stream of water 59, above and across the top surface of the work W to continuously deflect and remove slag resulting from the desurfacing operation. This nozzle is located 6 to 12 inches ahead of the nozzle head 12. This cross-fire water jet contributes greatly to the success of the operation.

A modification of the invention is shown in Fig. 6 which is identical in construction with the preferred embodiment hereinbefore described, except that in lieu of the flat slotted powder outlets 39 thereof, the modification employs round powder outlets 60. This construction is less expensive, does not clog up as readily and surprisingly functions just as well for the hot scarffing of stainless steel.

Another modification of the invention is shown in Fig. 7 in which the powder nozzle 10 identical with the preferred embodiment is mounted on a desurfacing head which, in lieu of the slotted nozzles 14, is provided with a transversely continuous slotted nozzle 62 having an oxygen slot 63 and upper and lower rows of preheat flame ports 64 and 65. The sheets of oxygen and powder laden gas have the same dihedral angle relation as in Fig. 2 and function in the same manner.

Fig. 8 shows the head of Figs. 1 and 2 arranged to scarf the four sides of rectangular work simultaneously. Inasmuch as the present invention is operative on the sides and bottom of the work, which has never been done heretofore on hot stainless steel, it is readily adapted for this simultaneous operation.

In operation, the mixture of air and powder from the dispenser 50 is passed through a suitable hose to the pinch valve 48, and thence through the booster 47 located immediately adjacent the dispenser, the purpose of the booster 47 being to increase the velocity of the air-powder mixture and make it airborne. This increase in velocity prevents the powder settling out by gravity in the horizontal run on the way from the dispenser 50. The booster 46 again increases the velocity of the air-borne powder stream and also sets up a turbulence which redistributes any powder settled out by centrifugal force in bends in the powder line, and causes the powder to be uniformly distributed in the tube leading to the distributor 44. From the distributor the air-borne powder mixture is equally divided among the multiple outlets 54, and passes on through the battery of equal tubes 42 onto the scarffing zone through the powder nozzle 10.

With the apparatus as above described, satisfactory hot scarffing was accomplished on the top, sides and bottom of stainless steel slabs and billets. It was further found that the slotted oxygen nozzle, the round orifice powder outlet, which is much simpler and cheaper than

the slotted type, produced equally as satisfactory a scarfed surface as the slotted type of powder orifice.

The advantages of hot machine scarffing of stainless steels with this equipment are as follows: A relatively smooth flat surface results which can readily be examined for deep seams or breaks and which will roll out into a satisfactory strip, sheet or plate mill product. Stainless steel was scarfed at speeds up to 120 feet per minute with no indication of loss of stability. With the preheat gases burning, starts can be made almost instantaneously with the turning on of the powder stream. The process is more efficient than cold scarffing from the standpoint of powder consumed. For cold scarffing powder consumption is on the order of 20 pounds per ton of steel; for hot scarffing according to the present invention on the order of two pounds per ton. Also, as to metal loss, it is easier to make a shallow cut—compared to cold scarffing, the metal loss is enormously reduced.

Important contributing factors to the successful operation of the process are: the powder distribution equipment which allows a single powder stream to be divided equally and directed over a multiplicity of scarffing nozzles or to a continuous oxygen slot. Also, a cross-fire water jet of high pressure water directed across the steel being scarfed transverse to the direction of scarffing to remove the slag from the surface of the steel before it has time to solidify. Without the cross-fire water jet it is difficult, if not impossible, to maintain a stable re-action.

30 The following are the operating conditions found to produce the most satisfactory surface on a 9½" width unit:

Depth of cut \_\_\_\_\_  $\frac{1}{32}$  inch.

Oxygen pressure \_\_\_\_\_ 45 pounds per square inch.

Table speed \_\_\_\_\_ 90 feet per minute—can be varied to

vary depth of cut.

Powder \_\_\_\_\_ 4 to 5 ounces per minute per scarffing nozzle, total 40 ounces per minute. Round orifice outlets inclined toward the work at an angle of 60°.

40 Nozzle height \_\_\_\_\_  $\frac{11}{16}$  inch.

Cross-fire water \_\_\_\_\_ Jets set to impinge approximately 8 in. in front of scarffing nozzle center line. Water pressure 80 to 100 pounds per square inch, delivering approximately 30 to 125 gallons per minute.

We claim:

50 1. Process of desurfacing a refractory metal body, which comprises applying preheat to a local surface portion of such body at substantially rolling temperature, discharging a relatively flat stream of oxidizing gas at an acute angle against such heated portion, separately passing a gas borne mixture of gas and adjuvant powder through a supply line to a distributor wherein it is divided into a plurality of separate paths, introducing additional gas under pressure to said supply line ahead of said distributor to increase the velocity of the gas borne powder stream prior to division thereof, discharging the gas borne powder from said paths through a row of separate outlets forming a separate relatively flat stream of gas containing uniformly transversely distributed powdered solid fuel at an acute angle toward such oxidizing gas stream, so that such streams form acute angles with one another and with such surface portion of the body, and relatively moving the body and such streams at substantially rolling speed so that successive surface portions thereof are progressively removed thermochemically by the combined scarffing action of the powdered solid fuel and the oxidizing gas stream.

60 2. Process of desurfacing a refractory metal body, which comprises applying preheat to a local surface portion of such body at substantially rolling temperature, discharging a relatively flat stream of oxidizing gas at

an acute angle against such heated portion, passing a separate stream of gas containing powdered solid fuel through a distributor wherein it is divided into a plurality of separate equal paths, discharging the gas-borne powder from said separate equal paths through a row of separate aligned outlets forming a relatively flat stream of gas-borne powder separate from and at an acute angle toward such oxidizing gas stream, so that such flat streams form dihedral angles with one another and with such surface portion of the body, and relatively moving the body and such streams at substantially rolling speed so that successive surface portions thereof are progressively removed thermochemically by the combined scarfing action of the powdered solid fuel and the oxidizing gas stream.

3. Process of desurfacing a refractory metal body, which comprises applying preheat to a local surface portion of such body at substantially rolling temperature, discharging a relatively flat stream of oxidizing gas at an acute angle against such heated portion, passing a mixture of gas and adjuvant powder from a dispenser through a supply line to a booster to increase the velocity of the gas-powder mixture and make it gas borne, passing the gas-borne mixture through a distributor wherein it is divided into a plurality of separate equal paths, and discharging the gas-borne powder from said separate equal paths through a row of spaced outlets forming a relatively flat stream of gas-borne powder separate from and at an acute angle toward such oxidizing gas stream, so that the central planes of such flat streams form acute angles with one another and with such surface portion of the body, and relatively moving the body and such streams at substantially rolling speeds so that successive portions thereof are progressively removed thermochemically by the combined scarfing action of the powdered solid fuel and oxidizing gas stream.

4. Apparatus for desurfacing a refractory metal body, which comprises means for applying preheat to a local surface portion of such body at substantially rolling temperature, means for discharging a relatively flat stream of oxidizing gas at an acute angle against such heated portion, means for separately passing a gas borne mixture of gas and adjuvant powder through a supply line to a distributor wherein it is divided into a plurality of separate paths, means for introducing additional gas under pressure to said supply line ahead of said distributor to increase the velocity of the gas borne powder stream prior to division thereof, means for discharging the gas borne powder from said paths through a row of separate outlets forming a separate relatively flat stream of gas containing uniformly transversely distributed powdered solid fuel at an acute angle toward such oxidizing gas stream, so that such streams form dihedral angles with one another and with such surface portion of the body, and means for relatively moving the body and such streams at substantially rolling speed so that successive surface portions thereof are progressively removed thermochemically by the combined action of the powdered solid fuel and the oxidizing gas stream.

5. Apparatus for desurfacing a refractory metal body, which comprises means for applying preheat to a local surface portion of such body at substantially rolling temperature, means for discharging a relatively flat stream of oxidizing gas at an acute angle against such heated portion, means for passing a separate stream of gas containing powdered solid fuel through a distributor wherein it is divided into a plurality of separate equal paths, means for discharging the gas-borne powder from said separate equal paths through a row of separate aligned outlets forming a relatively flat stream of gas-borne pow-

der separate from and at an acute angle toward such oxidizing gas stream, so that such flat streams form adjacent angles with one another and with such surface portion of the body, and means for relatively moving the body and such streams at substantially rolling speed so that successive surface portions thereof are progressively removed thermochemically by the combined scarfing action of the powdered solid fuel and the oxidizing gas stream.

- 10 6. Apparatus for desurfacing a refractory metal body, which comprises means for applying preheat to a local surface portion of such body at substantially rolling temperature, means for discharging a relatively flat stream of oxidizing gas at an acute angle against such heated portion, means for passing a mixture of gas and adjuvant powder from a dispenser through a booster to increase the velocity of the gas-powder mixture and make it gas borne, means for passing the gas-borne mixture through a distributor wherein it is divided into a plurality of separate equal paths, and means for discharging the gas-borne powder from said separate equal paths through a row of spaced outlets forming a relatively flat stream of gas-borne powder at an acute angle toward such oxidizing gas stream, so that the central planes of such flat streams form dihedral angles with one another and with such surface portion of the body, and means for relatively moving the body and such streams at substantially rolling speeds so that successive portions thereof are progressively removed thermochemically by the combined scarfing action of the powdered solid fuel and oxidizing gas stream.

- 15 7. Process of desurfacing a refractory metal body, which comprises applying preheat to a local surface portion of such body at substantially rolling temperature, 35 discharging a relatively flat stream of oxidizing gas at an acute angle against such heated portion, separately passing a gas borne mixture of gas and adjuvant powder through a supply line to a distributor wherein it is divided into a plurality of separate paths, introducing additional 40 gas under pressure to said supply line ahead of said distributor to increase the velocity of the gas borne powder stream prior to division thereof, discharging the gas borne powder from said paths through a row of separate outlets forming a separate relatively flat stream of gas containing uniformly transversely distributed powdered solid fuel at an acute angle toward such oxidizing gas stream, so that such streams form acute angles with one another and with such surface portion of the body, relatively moving the body and such streams at substantially rolling speed so that successive surface portions thereof are progressively removed thermochemically by the combined scarfing action of the powdered solid fuel and the oxidizing gas stream, and a stream of slag is formed and projected ahead of the reaction zone, and 50 discharging a stream of water transverse to the workpiece and ahead of the reaction zone to continuously deflect and remove such slag.

#### References Cited in the file of this patent

#### UNITED STATES PATENTS

|           |                 |               |
|-----------|-----------------|---------------|
| 2,327,337 | Burch et al.    | Aug. 24, 1943 |
| 2,451,422 | Wagner          | Oct. 12, 1948 |
| 2,465,297 | Thompson et al. | Mar. 22, 1949 |
| 2,470,999 | Meincke         | May 24, 1949  |
| 2,536,201 | Meincke et al.  | Jan. 2, 1951  |
| 2,538,074 | Anderson        | Jan. 16, 1951 |
| 2,622,048 | Moesinger       | Dec. 16, 1952 |
| 2,626,880 | Meincke         | Jan. 27, 1953 |